

Jan. 8, 1935.

W. D. KELLOGG

1,986,974

METHOD OF UNITING THREADS

Filed June 17, 1933.

Fig. 1.



Fig. 2.



Fig. 3.



Fig. 4.



Fig. 5.



INVENTOR  
William D. Kellogg  
BY  
Fannie Davis, Marion Edwards  
ATTORNEYS

## UNITED STATES PATENT OFFICE

1,986,974

## METHOD OF UNITING THREADS

William D. Kellogg, Amsterdam, N. Y., assignor  
to Mohawk Carpet Mills, Inc., Amsterdam,  
N. Y., a corporation of New York

Application June 17, 1933, Serial No. 676,285

6 Claims. (Cl. 28—1)

This invention relates to methods of uniting the ends of strands, such as threads, yarns, etc., and is concerned more particularly with a novel method of uniting strands without knotting or 5 tying and a new strand made up of smaller pieces united by that method. The method of the invention may be used to special advantage in the preparation and use of threads, yarns, etc. in the manufacture of textile fabrics, and the 10 adaptation of the invention to that field will accordingly be described in detail for purposes of explanation, although it is to be understood that the utility of the method is not limited to that specific application.

15 The breakage of threads and yarns occurs in all winding and spooling operations employed in the textile art and it is the usual practice to secure the ends together by tying. This operation is done either by hand or by a device known as a 20 hand-knotter, the latter being used when the strands are relatively small. The tying of the ends together results in the formation of an enlargement in the form of a knot in the strand and usually leaves two loose ends projecting from 25 the knot. The presence of such knots in threads and yarns causes many difficulties in weaving operations.

When warp threads break and are tied together, the resulting knots are frequently too 30 large to pass through the heddle eyes of the loom and through the spaces between the reed dents of the lay. When the knots reach the heddle eyes or reed dents, the threads are again broken, and this necessitates stopping the loom with a 35 consequent loss in loom efficiency. Even if the knots in the warp threads are small enough to pass through the heddle eyes and reed dent spaces, they are likely to cause lumps and imperfections in the body of the fabric which are 40 highly objectionable.

45 Knots in the pile yarn used in a carpet, rug, or similar fabric, produce serious defects, especially when they appear in the face yarn, and such knots must be removed by hand in a finishing operation which adds greatly to the cost of manufacture. The seriousness of the presence of knots in the pile yarn will be better appreciated when it is understood that in the weaving of a five frame Wilton rug of the 9' by 12' size, there is 50 a possibility of obtaining five thousand knots in the pile yarn alone, the majority of which must be removed, if a satisfactory pile surface is to be obtained.

55 Pile yarn knots present an equally serious problem in the weaving of Axminster fabrics. In

the ordinary Axminster looms in which each individual end of pile yarn is passed through a separate tube and presented to the fabric to be looped about a weft shot, such knots offer considerable resistance to the free passage of the 5 yarn through the tubes, and even though the knots are carefully made, they frequently cause breakage of the pile yarns and this requires the insertion of tufts by hand. Such operations reduce the loom efficiency materially and add 10 greatly to the cost of manufacture.

In fabrics in which the tufts are inserted by needles, the elimination of knots in the pile yarn is particularly important as each end of yarn must pass through a highly restricted space in 15 a hollow needle. If the knot is too large to pass through the space and a breakage of the thread results, the machine must be stopped and the needle rethreaded with resulting loss in time and production.

20 The essentials of any method by which the ends of threads or yarn are united and which is to be used in replacement for knotting either by hand or by machine are that the method must be at least as fast as tying a knot, and the 25 strength of the strand at the point of union must be equal to or greater than the strength of the individual threads. The method of the present invention fulfills these requirements and, in addition, the strand is flexible at the point of 30 union, the thickness is not increased over the original thickness of one end, and loose extremities of the strand do not extend from the point of union. The method of the present invention, therefore, offers great advantages over the method 35 of knotting or tying heretofore used and, when employed in connection with the production of fabrics, it results in increased efficiency in weaving and knitting operations and in a reduction 40 in the cost of finishing.

45 The method of the present invention depends on the use of an adhesive which sets rapidly, and in practicing the invention, the ends of the strands to be united are placed in substantial alignment, preferably with a slight overlap, a quantity of adhesive is applied to the ends, and the ends are then pressed together. During the pressing operation, the mass of adhesive is shaped so that it forms a coating or sheath for the ends, this sheath being substantially of the same diameter as one of the ends. The new method can be most conveniently carried out by hand, a drop of the adhesive being applied to the forefinger, the ends then being rolled in contact with one another and with the adhesive by 50

means of the thumb and forefinger. The pressing and rolling operations can be performed mechanically, if desired, but manual operations are entirely satisfactory and are preferred.

- 5 The new strand made up of two or more pieces connected together in accordance with the new method has no enlargements and is flexible at the points of union. The connections are fully as strong as knots and there are no loose ends projecting from the connections.

10 For a better understanding of the invention, reference may be had to the accompanying drawing, in which

15 Figure 1 illustrates the first step in the new method carried out by hand;

Figure 2 illustrates the second step;

Figure 3 illustrates the third step, and

20 Figures 4 and 5 are views in section and elevation, respectively, of the union of a pair of strands made by the new method.

In carrying out the new method by hand, a small quantity such as a good sized drop 10 of the adhesive is placed on the forefinger 11, and the ends 12 and 13 of the strands to be united are 25 then placed in substantial alignment and preferably with a slight overlap in contact with the drop of adhesive. The thumb 14 is then placed on top of the ends of strands and the thumb and forefinger moved relatively so that the ends of the 30 strands are rolled across the adhesive.

The application of pressure by this rolling operation is continued until the adhesive sets and in the operation, the adhesive impregnates the fibres of the strands and also coats them. If 35 the proper type of adhesive is employed, it passes completely from the finger to the ends of the strands and both impregnates and coats the fibres so that at the point of union, the ends of the strands are encased in a continuous sheath 15.

40 The adhesive which I have found to give the best results for the purpose is a latex from the *Hevea brasiliensis* tree which has been concentrated to bring the dry rubber content to approximately 50% to 65% by weight and which has 45 been preserved by the addition of a small amount of ammonia such as 1% to 3%. Ammonia in this amount serves to preserve the latex and retard coagulation, but when such a latex is subjected to a slight pressure and rolling action, it 50 coagulates readily, the ammonia being volatilized by that action. A small amount of an anti-oxidant and an accelerator can also be added if desired but these additions are not absolutely essential in order that the latex may serve the desired purpose.

55 The method of concentrating the latex which I prefer is one which will leave the concentrate practically free from the non-rubber constituents of the natural latex and in a comparatively unstable and sensitive condition such that when the latex is subjected to a relatively slight pressure and rolling action, it will be converted into an irreversible coagulum.

60 The methods of concentration which have been 65 found satisfactory for placing the latex in the desired condition are those in which the greater part of the non-rubber constituents or the natural protective colloids are eliminated from the natural latex and in which no protective colloids are added to retard coagulation. Preferably, the methods of concentration by creaming or centrifuging are employed.

65 In the method of concentrating the latex by creaming, small quantities of a vegetable mucus, such as Iceland moss, are added to the natural

70 latex and the mixture is allowed to stand for a time, heat being applied if desired to accelerate the separation. The rubber particles of the latex concentrate in a top layer which can be drawn off while the water and the water soluble compounds comprising the non-rubber constituents 75 form the lower layer.

75 The method of centrifuging depends on the 80 mechanical separation of the latex by centrifugal action into a cream and a skimmed milk. The cream contains a high percentage of rubber and the skimmed milk a low percentage of rubber together with practically all of the non-rubber constituents.

85 Other methods can also be employed such as 90 filtration, these methods resulting in the removal of the water and water solubles and leaving a concentrate which contains a relatively high percentage of rubber particles and only a small percentage of the non-rubber constituents.

95 In the use of any of the methods mentioned, the purpose is to concentrate the latex so that the resulting product contains a percentage of rubber particles higher than that in the natural latex and a percentage of non-rubber particles lower 100 than that in the natural latex. I have found that the latex containing 50% to 65% dry weight of rubber particles and containing 1% to 3% of ammonia is most satisfactory in the uniting of strands in accordance with the new method.

105 When a drop of this material is placed on the forefinger and the ends of the strands rolled together with the drop in the manner above described, rapid coagulation of the latex occurs and the operation consumes no more time than the 110 ordinary tying of a knot. In addition, the rolling action so distributes the latex that there is no lump or enlargement at the point of union and the film or sheath of latex which secures the ends of the strand together is flexible and the union 115 has at least the strength of a single strand.

120 What I claim is:

1. A method of uniting a pair of strands which comprises applying to the portions of said strands to be united, a quantity of rubber latex containing a small amount of a preservative compound, 125 said latex being in sensitive and unstable condition and having the property of coagulating rapidly when a small quantity thereof is rolled and pressed in the air, and pressing said portions 130 and latex together with a rolling motion continuing until said latex coagulates.

135 2. A method of uniting a pair of strands which comprises applying to portions of said strands to be united latex containing from about 50% to 140 about 65% by weight of dry rubber content and a small amount of a preservative compound, and pressing and rolling said portions together until said latex coagulates.

145 3. A method of uniting a pair of strands which comprises applying to portions of said strands to be united concentrated latex containing an 150 unnaturally high percentage of rubber particles, an unnaturally small amount of non-rubber constituents, and a small amount of a preservative compound, and pressing and rolling said portions together until said latex coagulates.

155 4. A method of uniting a pair of strands which comprises applying to portions of said strands to be united latex containing rubber in excess of the natural amount and a small amount of a volatile preservative compound, said latex being in sensitive and unstable condition and having the property of coagulating rapidly when a small quantity thereof is rolled and pressed in the air,

and pressing and rolling said portions together with the latex until coagulation of the latex occurs.

5. A method of uniting a pair of strands which comprises applying rubber latex containing a small amount of a volatile coagulation retarder to the portions of said strands which are to be united, said latex having the property of coagulating rapidly when a small quantity thereof is 10 rolled and pressed in the air and maintaining said portions in contact until said latex has coagulated.

6. A method of uniting a pair of strands which comprises applying to the portions of said strands which are to be united a concentrated rubber latex containing an unnaturally small amount of non-rubber constituents and a protective compound, said latex having the property of coagulating rapidly when rolled and pressed in the air, and applying pressure to hold said portions in contact until said latex has coagulated.

5

10

WILLIAM D. KELLOGG.